

# UNITED STATES PATENT OFFICE.

ROBERT ATHELSTAN MARR, OF NORFOLK, VIRGINIA, ASSIGNOR TO AMERICAN WOOD  
ENCYSTING CO., INCORPORATED, OF NORFOLK, VIRGINIA, A CORPORATION OF  
VIRGINIA.

## PRESERVED WOOD AND METHOD OF MAKING SAME.

1,121,646.

Specification of Letters Patent. Patented Dec. 22, 1914.

No Drawing. Original application filed February 8, 1913, Serial No. 747,169. Divided and this application filed January 13, 1914. Serial No. 811,914.

*To all whom it may concern:*

Be it known that I, ROBERT ATHELSTAN MARR, a citizen of the United States, residing at Ghent, Norfolk, in the county of Norfolk and State of Virginia, have invented certain new and useful Improvements in Preserved Wood and Methods of Making Same, of which the following is a specification.

10 My present invention relates to certain improvements in the process of encysting wood.

In my U. S. Patent No. 1,023,745, dated April 16, 1912, I have described a process 15 which consists essentially in that the wood to be treated is first soaked in a volatile hydrocarbon, such as gasolene, after which it is immersed in a bath containing melted paraffin and diatomaceous earth, which mixture enters the pores, ducts and cells of the timber and thoroughly permeates and encysts these. In my other U. S. Patent No. 1,023,784, dated April 16, 1912, I have described a process in which timber is 20 immersed in a bath of molten paraffin and naphthalene, which materials enter and encyst the pores, ducts and sap channels of the wood.

The process of the present application 30 combines features of both these processes, and is carried out preferably in the following manner: Wood is immersed in a bath containing a mixture of paraffin, naphthalene and Paris green, with or without diatomaceous earth, while said bath is at a temperature somewhat above the boiling point of water, a temperature of near 240° F. being preferred. The temperature should not be carried very much above this limit, since at 35 higher temperatures the strength of the wood may be impaired. The air and moisture in the ducts of the wood are driven out by the action of the naphthalene in the bath, and the melted mixture, carrying the diatomaceous earth, rapidly enters and takes its 40 place, and thoroughly encysts the pores and ducts of the wood.

The bath is preferably composed of the materials in the following proportions (by weight) although the invention is not limited thereto, paraffin, 100 parts; naphtha-

lene 5 to 15 parts, Paris green, 1 part, to which diatomaceous earth, 2 to 5 parts, may be added if desired.

In carrying out this process any variety 55 of wood may be thoroughly permeated by the mixture, from center to circumference, such woods as beach, pine, oak, gum, Douglas fir, etc., many of which cannot be impregnated by the ordinary vacuum and pressure process, using hot creosote, except very superficially, and moreover several kinds of wood may be treated simultaneously in the same bath, and the wood may be in either a horizontal or vertical or inclined position. 60

When it is desired to treat a part only of the length of a stick, for example a pile, it may be stood up on end, in a tank containing the mixture, in which case the paraffin and naphthalene will thoroughly permeate 70 the wood of the length actually immersed, and some distance beyond, being carried up some distance, within the wood, above the surface of the bath.

Bent samples of the various hard and soft 75 woods, both green and dry have been treated, in accordance with my present invention, with only a sector of the bent portion immersed; the encysting mixture thoroughly impregnates the wood where immersed and 80 is carried up considerable distance toward each end.

It is to be noted that either green or seasoned wood may be treated, and the impregnation, when using green wood is not only 85 as complete as when using dry wood, but it takes places in a shorter time, and both green and dry wood may be treated together, in the same bath. Another point of great value is the fact that wood with the bark on, or sawed timber may be treated equally well, and in both these cases absolutely complete 90 impregnation can be secured. This is particularly surprising in using such wood as Southern pine, which, in order to be creosoted must not only have its outer bark removed, but also the inner bark or skin must also be substantially completely removed, since creosote, even hot and under heavy 95 pressure cannot pass through this inner bark or skin, as has been repeatedly demonstrated, to the sorrow of many firms attempting to

impregnate this variety of wood with creosote, by the well-known vacuum and pressure processes.

The use of a temperature of somewhat 5 above the boiling point of water, in place of somewhat below, as in my processes in the patents above referred to, makes the action take place in very much less time, and consequently saves time and money in the 10 operation of the process, and accelerates the action of the preservative on the wood.

I find that in some instances it is neither necessary nor desirable to lower the temperature of the bath before removing the wood 15 therefrom. Accordingly the bath may be maintained at a uniform temperature, as nearly as possible, wood being immersed and taken out when impregnated, and then more wood immersed. The absorption of 20 the material by the wood is compensated for by suitable additions of the materials to the bath, from time to time, as necessary.

It is easy to see when the impregnation 25 and encysting is complete, as no more bubbles are given off from the surface of the wood.

If it is desired to supersaturate the treated material and leave the main ducts and pores completely filled a drop in temperature 30 is preferable, or the timber may be immersed in another similar bath at a lower temperature.

The apparatus preferably used, in carrying 35 out my process is an open tank with heating means, such as steam coils therein, and it is unnecessary to employ vacuum or pressure in carrying out the process, which also effects a great saving in the process.

On account of the fact that the bubbles of 40 air and steam coming out of the wood, will in most cases, keep the bath sufficiently agitated, it is not ordinarily necessary to provide stirring means. However, stirring means may in some instances be advisable.

45 The diatomaceous earth is an extremely finely divided material, of which over 90% will pass through the meshes of a sieve or bolting cloth having 40,000 meshes per square inch, and this is carried by the melted paraffin into the interior of the wood. The function of this, as in my prior patent, is to leave a hard solid material in the interstices of the wood which will prevent the 50 action of teredo, limnoria, etc., whose mandibles are composed essentially of carbonate of lime (a material much softer than the silica of which the diatoms are composed). And the magma adds strength and resiliency to treated woods.

60 The Paris green while a fine powder, is much coarser than the diatomaceous earth, and consequently does not enter the wood to any great extent, but remains as a coating, on, and somewhat beneath the surface 65 of the wood. This will effectually prevent

the action of wood-destroying insects, also most forms of wood destroying fungi, since as well known it is a poison to both insect life and fungi.

The paraffin acts to prevent the entrance 70 of moisture, fungi, spores, and acts as a preservative to the timber, since wood cannot decay in the absence of water. It is very difficult to impregnate wood with ordinary paraffin, in a molten condition, since 75 this paraffin merely forms a coating over the surface of the wood, and does not enter the minute cells and cavities of the wood. I have, however, found that the addition of naphthalene acts as a carrier, to cause the 80 paraffin to readily be carried into the smallest pores and cavities of the wood being treated. This may be due to the fact that the naphthalene is somewhat volatile, and in starting to vaporize it drives out the 85 moisture, or air in the wood, and then the paraffin enters. Moreover the naphthalene cleans out the tissue ducts of the timber, to make it possible for the mixture to enter.

The wood when treated according to this 90 process is also stronger and heavier than before treatment, which is also a valuable feature of the process.

Wood, when encysted according to my present process, will effectually resist any 95 form of wood destroying fungus, insect, worm, or any form of decay.

It is obvious that in place of naphthalene, I can employ other aromatic hydrocarbons of this type, which are somewhat volatile, 100 such as homologues or naphthalene, may be employed. Also in place of paraffin, other non-volatile materials, which are insoluble in water, and which are capable of being melted, and which when so melted will form 105 thin liquids of a mobile nature, at the temperatures mentioned herein. Various equivalents for the diatomaceous earth, and for the Paris green may also be used.

The strength and resiliency of the wood, 110 are in all cases increased, the reason probably being that the silica forms with the paraffin, a magma, which upon cooling solidifies within the ducts of the wood to produce a supporting cylinder therein. 115

This application is a division of my co-pending application, Serial No. 747,169, filed Feb. 8, 1913.

The treatment of certain varieties of 120 wood, with mixtures such as are herein described, is claimed in my copending applications, Serial Numbers 811,909 and 811,910, filed concurrently herewith. The treatment of wood with paraffin, diatomaceous earth and naphthalene is claimed in the parent 125 case above referred to.

What I claim is:

1. A process of preserving wood, which comprises immersing said wood in a bath 130 containing a non-volatile, water-insoluble

material solid at ordinary temperature, said material having a melting point not over 212° F.; a somewhat volatile hydrocarbon of the aromatic series; and an insoluble insecticidal body.

2. A process of preserving wood, which comprises immersing said wood in a bath containing normally solid paraffin, naphthalene and Paris green at substantially 10 atmospheric pressure.

3. A process of preserving wood, which comprises immersing said wood in a bath containing normally solid paraffin, naphthalene and Paris green; at a temperature 15 somewhat above the boiling point of water, and thereafter allowing said bath to cool to a temperature below the boiling point of water.

4. A product consisting of wood, the

pores, ducts and cells of which are encysted 20 with a solid mixture comprising solid paraffin, and an aromatic hydrocarbon, said wood having a coating comprising a water-proof layer including solid paraffin, and an insoluble insecticidal body.

5. A product consisting of wood, the 25 pores, ducts and cells of which are encysted with a solid mixture comprising paraffin and an aromatic hydrocarbon, said wood being coated with a mixture, including 30 solid paraffin and Paris green.

In testimony whereof I have affixed my signature in presence of two witnesses.

ROBERT ATHELSTAN MARR.

Witnesses:

JANEY HOPE MARR,  
A. B. FOSTER.